

# United States Patent Office

3,375,114

Patented Mar. 26, 1968

1

3,375,114  
HIGH EDGE GRADIENT SILVER  
HALIDE EMULSION

Yoshihide Hayakawa and Yosuke Nakajima, Minamishigara-machi, Japan, assignors to Fuji Photo Film Co., Ltd., Kanagawa-ken, Japan, a corporation of Japan  
No Drawing, Filed Mar. 29, 1965, Ser. No. 443,662  
Claims priority, application Japan, Dec. 26, 1961,

37/47,418

6 Claims. (Cl. 96—107)

This invention relates to a photographic emulsion of silver halide and more particularly to a photographic emulsion giving an image of high edge gradient.

The ratio of change in density to distance at the boundary between the darkened part and the undarkened part of a photographic image is called "edge gradient." In general, the higher the edge gradient, the sharper the image. In order to obtain an image of high edge gradient, a special developing solution which contains a small amount of sulfite salt, having a high pH value and containing hydroquinone alone as developer, has been employed (for example, ref. Yule, J.A.C., "Formaldehyde-Hydroquinone Developers and Infectious-Development," J. Frank. Inst., 239,221 (1945)).

It is the object of this invention to provide a photographic emulsion which gives an image of high contrast when a developing solution of this type is employed.

Photosensitive materials using such emulsion are suitable for making the half-tone reproductions by means of reproduction screens such as glass screen and contact screen. The above-mentioned object can be attained by adding to the emulsion (1) the derivatives of 4-hydroxy-1,3,3a,7-tetraazaindene and (2) at least one compound selected from the group consisting of lysine and arginine and their salts. The derivatives of 4-hydroxy-1,3,3a,7-tetraazaindene are represented by the following structural formula:



where R and R<sub>1</sub> represent hydrogen atom, alkyl group, aralkyl group or aryl group, and R<sub>2</sub> represents hydrogen atom, alkyl group, carboxy group or carboalkoxy group.

The derivatives of tetraazaindene capable of being employed in this invention can be synthesized by heating 1 mole of  $\beta$ -ketoesters, malonic esters of  $\alpha$ -ethoxymethylene- $\beta$ -ketoesters with 1 mole of 3-amino-1,2,4-triazoles. Examples of such tetraazaindene are as follows:



2



(IV)

Additional examples of tetraazaindenes are as follows:



Lysine and arginine used in this invention are basic amino-acids, and both that prepared by the decomposition of proteins and that prepared by synthesis may be employed. These compounds are represented by the following structural formulae:

Lysine (hydrochloride)



(V)



(VI)

The amount of compounds employed in this invention varies according to the sort of emulsion, but it is preferable to add 10 mg. to 1 g. of tetraazaindene, 0.1 g. to 10 g. of lysine or arginine or their salts per 1 mole of silver halide.

Photographic emulsions are prepared in the following three stages: (1) The emulsification and digestion (first ripening) of the silver halide, (2) removal of excess of salts by washing with water and the like, and (3) second digestion (after ripening) to increase the sensitivity. The compounds may be added at any stage. Tetraazaindene may be added either before or after the addition of lysine or arginine, but it is most preferable to add these substances after the second ripening and before coating. These substances are dissolved in the solvents that have no detrimental effect on the emulsion, for example, water, lower alcohols such as methanol and ethanol, and ketones, and then added to the emulsion.

In this invention an emulsion of silver chloride, silver bromide, silver chlorobromide, silver iodo bromide, or silver chloroiodo bromide may be employed, but that of silver chlorobromide is most preferable.

The emulsion may be chemically sensitized by unstable compounds containing sulfur, such as ammonium thio-



consisting of 4-hydroxy-1,3,3a,7-tetrazaindenes which are represented by the following structural formula:



in which R and R<sub>1</sub> represent a member selected from the group consisting of hydrogen atom and alkyl groups and R<sub>2</sub> represents a member selected from the group consisting of hydrogen atom, alkyl groups, carboxy groups, and carboalkoxy groups, and (2) at least one compound se-

lected from the group consisting of lysine, arginine and their salts.

5. A method according to claim 4 wherein said compound (2) is lysine hydrochloride.

6. A method according to claim 4 wherein said compound (2) is arginine hydrochloride.

#### References Cited

#### UNITED STATES PATENTS

10 2,944,902 7/1960 Carroll et al. \_\_\_\_\_ 96—107

NORMAN G. TORCHIN, *Primary Examiner.*

G. COHN, *Assistant Examiner.*